

# UNITED STATES PATENT OFFICE.

MAX BAZLEN AND THEODOR WOHLFAHRT, OF LUDWIGSHAFEN-ON-THE-RHINE, GERMANY,  
ASSIGNORS TO BADISCHE ANILIN & SODA FABRIK, OF LUDWIGSHAFEN-ON-THE-RHINE,  
GERMANY, A CORPORATION.

## PROCESS OF MAKING STABLE ZINC HYDROSULFITE.

No. 896,610.

Specification of Letters Patent. Patented Aug. 18, 1908.

Application filed October 3, 1907. Serial No. 395,791.

To all whom it may concern:

Be it known that we, MAX BAZLEN and THEODOR WOHLFAHRT, doctors of philosophy and chemists, subjects, respectively, of the King of Württemberg and the King of Bavaria, residing at Ludwigshafen-on-the-Rhine, Germany, have invented new and useful improvements in Processes of Making Stable Zinc Hydrosulfite, of which the following is a

specification.

In the *Wiener Monatshefte*, Vol. 20, page 681, is described the production of solid zinc hydrosulfite by reacting with sulfur dioxid on zinc, in the presence of alcohol. The author poured absolute alcohol (which had been distilled several times over sodium) onto granulated zinc and then passed in sulfur dioxid, while cooling in order to prevent decomposition of the zinc salt formed. The zinc hydrosulfite is thus obtained in the form of long needle-like crystals, and is unstable, as, even when in closed vessels, it evolves sulfur dioxid after a few days, while in the presence of the atmosphere, its reducing power diminishes rapidly and it is therefore (in common with zinc hydrosulfite which has been prepared in aqueous solution) unsuitable for use in manufactures.

We have discovered that by passing a current of sulfur dioxid into a mixture of zinc dust and alcohol at a temperature above 40° centigrade (preferably between 60° and 75° centigrade) zinc hydrosulfite is obtained which possesses excellent keeping properties.

In carrying out our invention either absolute, or diluted, alcohol can be employed. When diluted alcohol is used, it is preferred to use such a concentration that the zinc hydrosulfite formed remains, as far as possible, undissolved. The zinc hydrosulfite is obtained, in almost theoretical yield, and is in the form of large six-sided, transparent leaflets, and, after drying, for instance *in vacuo*, is of excellent stability.

Either ethyl alcohol, or other alcohols, such for instance as methyl-alcohol, amyl-alcohol, and glycerin, and also other liquids

which substantially prevent the zinc hydrosulfite from going into solution, can be employed in carrying out this invention.

The following is an example of how our invention can be carried into practical effect, but it is not confined to this example. The parts are by weight. Allow four hundred and seventy (470) parts of sulfur dioxid to react on a mixture of six hundred (600) parts of methylated spirits, two hundred and fifty (250) parts of water and two hundred and seventy (270) parts of zinc dust, at a temperature of from sixty (60), to seventy-five (75), degrees centigrade, while well stirring the mixture. A paste of crystalline zinc hydrosulfite is thereby obtained. Filter this off, and wash it with methylated spirits and dry it *in vacuo* at a temperature of from sixty (60), to seventy (70), degrees centigrade, the zinc hydrosulfite being thus obtained in the condition of dry powder.

Now what we claim is:

1. The process of producing stable solid zinc hydrosulfite by passing a current of sulfur dioxid into a mixture of zinc dust and a liquid which substantially prevents the zinc hydrosulfite from going into solution, at a temperature above forty degrees centigrade. 75

2. The process of producing stable solid zinc hydrosulfite by passing a current of sulfur dioxid into a mixture of zinc dust and alcohol at a temperature above forty degrees centigrade. 80

3. The process of producing stable solid zinc hydrosulfite by passing a current of sulfur dioxid into a mixture of zinc dust and ethyl alcohol at a temperature between sixty and seventy-five degrees centigrade. 85

In testimony whereof we have hereunto set our hands in the presence of two subscribing witnesses.

MAX BAZLEN.  
THEODOR WOHLFAHRT.

Witnesses:

ERNEST F. EHRHARDT;  
J. ALEX. LLOYD.